# EUROPEAN PATENT SPECIFICATION

(11) **EP 0 258 288 B1**
(45) Date of publication and mention of the grant of the patent: **08.05.1991**
(21) Application number: 87900926.4
(22) Date of filing: 08.01.1987
(51) Int. Cl.: G03C 7/30

(54) **PHOTOGRAPHIC COLOR DEVELOPING COMPOSITIONS WHICH ARE ESPECIALLY USEFUL WITH HIGH CHLORIDE PHOTOGRAPHIC ELEMENTS**
PHOTOGRAPHISCHE FARBENTWICKLUNGSZUBEREITUNGEN ZUR VERWENDUNG INSBESONDERE BEI PHOTOGRAPHISCHEN ELEMENTEN MIT HOHEM CHLORIDGEHALT
COMPOSITIONS PHOTOGRAPHIQUES DE DEVELOPPEMENT EN COULEUR, SPECIALEMENT UTILES AVEC DES ELEMENTS PHOTOGRAPHIQUES A HAUTE TENEUR EN CHLORURE

(30) Priority: 24.01.1986 US 822097
(43) Date of publication of application: 09.03.1988
(73) Proprietor: EASTMAN KODAK COMPANY, Rochester, New York 14650-2201 (US)
(72) Inventor: VINCENT, Sheridan, E., Rochester, NY 14615 (US); BERLS, Richard, W., Rochester, NY 14617 (US)
(74) Representative: Buff, Michel
(86) International application number: US8700021
(87) International publication number: WO8704534

(56) References cited:
- EP-A- 211 437
- CH-A- 474 093
- DE-A- 2 740 322
- FR-A- 2 200 546
- FR-A- 2 394 113
- GB-A- 2 059 616
- Research Disclosure, no. 190, Feb. 1980, ( Industrial Opportunities, Havant, Hampshire, GB ), R.O. Deegan et al., "Control of microbiological growth in black-and-white photographic developers" , page 58, no. 19006, see the whole item

## Description

### FIELD OF THE INVENTION

This invention relates in general to photography and in particular to novel compositions and methods for processing photographic color elements. More specifically, this invention relates to novel photographic color developing compositions and to a novel method of rapid access processing of high chloride photographic elements utilizing such developing compositions.

### BACKGROUND OF THE INVENTION

The formation of color photographic images by the image-wise coupling of oxidized primary aromatic amino developing agents with color forming or coupling compounds to form indoaniline, indophenol, and azomethine dyes is well known. In these processes, the subtractive process of color formation is ordinarily used, and the image dyes customarily formed are cyan, magenta, and yellow, the colors that are complementary to the primary colors, red, green, and blue, respectively. Usually phenol or naphthol couplers are used to form the cyan dye image; pyrazolone or cyanoacetyl derivative couplers are used to form the magenta dye image; and acylacetamide couplers are used to form the yellow dye image.

In these color photographic systems, the color-forming coupler may be either in the developer solution or incorporated in the light-sensitive photographic emulsion layer so that, during development, it is available in the emulsion layer to react with the color developing agent that is oxidized by silver image development. Diffusible couplers are used in color developer solutions. Nondiffusing couplers are incorporated in Photographic emulsion layers. When the dye image formed is to be used in situ, couplers are selected which form non-diffusing dyes. For image transfer color processes, couplers are used which will produce diffusible dyes capable of being mordanted or fixed in the receiving sheet.

Photographic color elements often utilize silver halide emulsions of the high bromide type, including silver bromide, silver bromoiodide and silver chlorobromide emulsions. However, as explained in Atwell, United States patent 4,269,927, issued May 26, 1981, high chloride silver halide photographic elements _ that is, elements in which the silver halide grains are at least 80 mole percent silver chloride _ possess a number of highly advantageous characteristics. For example, silver chloride possesses less native sensitivity in the visible region of the spectrum than silver bromide, thereby permitting yellow filter layers to be omitted from multicolor photographic elements. Furthermore, high chloride silver halides are more soluble than high bromide silver halides, thereby permitting development to be achieved in shorter times.

Photographic color developing compositions used heretofore have typically been adapted for use with high bromide silver halide photographic elements. These conventional developing compositions can be used with high chloride silver halide photographic elements, but, in general, they tend to give less than satisfactory results. For example, they typically contain restraining agents such as potassium bromide, which exert too great a retardation effect on development for satisfactory use with high chloride silver halide elements. Moreover, they typically contain hydroxylamine, or a water-soluble acid salt thereof, which functions as an anti-oxidant and thereby serves to protect the primary aromatic amino color developing agent against oxidation. Use of hydroxylamine, or a water-soluble acid salt thereof, is disadvantageous, however, since it tends to act as a scavenger which reduces oxidized color developing agent before it can react with coupler to form dye. It also acts as a developing agent which competes with the color developing agent unless it is adequately restrained by bromide. In addition to hydroxylamine, or a water-soluble acid salt thereof, developing compositions heretofore used with high bromide silver halide elements often contain substantial concentrations of sulfite to also provide protection against oxidation of the developing agent. The sulfite, which is typically utilized in the form of an alkali metal sulfite or bisulfite, functions to sulfonate oxidized color developing agent and, when used in sufficient concentration, its competition with coupler for oxidized color developing agent seriously affects dye formation.

Included among the numerous patents which describe photographic color developing compositions, of the type typically used with high bromide silver halide elements, are the following:
Kridel, U.S. patent 2,875,049, issued February 24, 1959,
Tassone, U.S. patent 3,462,269, issued August 19, 1969,
Anselm, U.S. patent 3,489,566, issued January 13, 1970,
Heilmann, U.S. patent 3,746,544, issued July 17, 1973,
Brown, U.S. patent 3,839,045, issued October 1, 1974,
Frank, U.S. patent 3,994,730, issued November 30, 1976,
Shimamura et al, U.S. patent 4,083,723, issued April 11, 1978,
Case et al, U.S. patent 4,170,478, issued October 9, 1979,
Case, U.S. patent 4,252,892, issued February 24, 1981,
Vincent et al, U.S. patent 4,264,716, issued April 28, 1981,
Cappel, U.S. patent 4,394,440, issued July 19, 1983,
Kapecki et al, U.S. patent 4,414,307, issued November 8, 1983,

Twist et al, U.S. patent 4,482,626, issued November 13, 1984.

In light of the above, it is clear that there is a need in the art to provide photographic color developing compositions and photographic processes which are especially adapted for use with high chloride silver halide elements if the inherent advantages of such elements are to be most fully realized. It is toward the objective of filling such need that the present invention is directed.

### SUMMARY OF THE INVENTION

The novel photographic color developing compositions of this invention are especially useful with high chloride silver halide emulsions. They are free, or at least substantially free, of bromides, since bromides in significant quantities can unduly restrain the development reaction. They are free of sulfite, or contain only a low concentration of sulfite, to minimize competition with the dye-forming reactions. They contain the following ingredients:
(1) a primary aromatic amino color developing agent,
(2) an N,N-dialkylhydroxylamine,
(3) at least one sequestering agent which functions to sequester iron,
(4) at least one sequestering agent which functions to sequester calcium, and
(5) from zero to 0.2 moles of sulfite per mole of said primary color developing agent.

In a preferred embodiment of the invention, the aforesaid photographic color developing composition is free of benzyl alcohol and is used in a rapid access process for processing high chloride silver halide photographic color elements which employs the steps of color developing, bleach-fixing without washing between the color developing and bleach-fixing steps, and stabilizing without washing between the bleach-fixing and stabilizing steps. Elimination of the benzyl alcohol from the developing composition allows the bleach-fix to be utilized at a lower pH than is otherwise permissible, without the risk of producing leuco cyan dye. The low pH increases the rate of bleach-fix reactions, thereby enabling the use of a short bleach-fix time as is needed for a rapid access process.

### DESCRIPTION OF THE PREFERRED EMBODIMENTS

The primary aromatic amino color developing agents that are utilized in the compositions and methods of this invention are well known and widely used in a variety of color photographic processes. They include aminophenols and p-phenylenediamines. They are usually used in the salt form, such as the hydrochloride or sulfate, as the salt form is more stable than the free amine, and are generally employed in concentrations of from about 0.1 to about 20 grams per liter of developing solution and more preferably from about 0.5 to about 10 grams per liter of developing solution.

Examples of aminophenol developing agents include o-aminophenol, p-aminophenol, 5-amino-2-hydroxy-toluene, 2-amino-3-hydroxy-toluene, 2-hydroxy-3-amino-1,4-dimethylbenzene, and the like.

Particularly useful primary aromatic amino color developing agents are the p-phenylenediamines and especially the N,N-dialkyl-p-phenylenediamines in which the alkyl groups or the aromatic nucleus can be substituted or unsubstituted. Examples of useful p-phenylenediamine color developing agents include:
N,N-diethyl-p-phenylenediamine monohydrochloride,
4-N,N-diethyl-2-methylphenylenediamine monohydrochloride,
4-(N-ethyl-N-2-methanesulfonylaminoethyl)-2-methylphenylenediamine sesquisulfate monohydrate,
4-(N-ethyl-N-2-hydroxyethyl)-2-methylphenylenediamine sulfate,
4-N,N-diethyl-2,2′-methanesulfonylaminoethylphenylenediamine hydrochloride.

An especially preferred class of p-phenylenediamine developing agents are those containing at least one alkylsulfonamidoalkyl substitutent attached to the aromatic nucleus or to an amino nitrogen. Other especially preferred classes of p-phenylenediamines are the 3-alkyl-N-alkyl-N-alkoxyalkyl-p-phenylenediamines and the 3-alkoxy-N-alkyl-N-alkoxy-alkyl-p-phenylenediamines. These developing agents are described in United States Patents 3,656,950 and 3,658,525, and can be represented by the formula:
wherein n is an integer having a value of from 2 to 4, R is an alkyl group of from 1 to 4 carbon atoms, and R¹ is an alkyl group of from 1 to 4 carbon atoms or an alkoxy group of from 1 to 4 carbon atoms. Illustrative examples of these developing agents include the following compounds:
N-ethyl-N-methoxybutyl-3-methyl-p-phenylenediamine,
N-ethyl-N-ethoxyethyl-3-methyl-p-phenylenediamine
N-ethyl-N-methoxyethyl-3-n-propyl-p-phenylenediamine,
N-ethyl-N-methoxyethyl-3-methoxy-p-phenylenediamine,
N-ethyl-N-butoxyethyl-3-methyl-p-phenylenediamine.

In addition to the primary aromatic amino color developing agent, the developing compositions of this invention contain an N,N-dialkylhydroxylamine. The N,N-dialkylhydroxylamine can be used in the color developing composition in the form of the free amine, but is more typically employed in the form of a water-soluble acid salt. Typical examples of such salts are sulfates, oxalates, chlorides, phosphates, carbonates, acetates, and the like.

The N,N-dialkylhydroxylamine is preferably of the formula:
wherein R³ and R⁴ represent the same or different alkyl groups of 1 to 4 carbon atoms.

Typical examples of N,N-dialkylhydroxylamines include:
N,N-diethylhydroxylamine,
N-ethyl-N-methylhydroxylamine,
N-ethyl-N-propylhydroxylamine,
N,N-dipropylhydroxylamine,
N-methyl-N-butylhydroxylamine.

Using the N,N-dialkylhydroxylamine in the photographic color developing compositions of this invention provides fully adequate stability against oxidation, without the unwanted development and unwanted reaction with oxidized color developing agent that occurs with the use of unsubstituted hydroxylamines or mono-alkyl substituted hydroxylamines. This is believed to be a result of the two alkyl groups attached to the nitrogen atom serving to block the site at which reaction could otherwise take place.

N,N-dialkylhydroxylamines have been used heretofore in photographic color developing compositions. Thus, for example, they are used in the magenta color developing solutions described in Anselm, United States patent 3,489,566, issued January 13, 1970. However, in these magenta developing solutions, they are employed in combination with an unsubstituted or mono-alkyl substituted hydroxylamine, and they serve as balancing developing agents.

As described hereinabove, the novel color developing compositions of this invention contain at least one sequestering agent which functions to sequester iron. The preferred sequestering agent for this purpose is an aromatic polyhydroxy compound that forms a complex with ferric ion in alkaline solution in which the molar ratio of the ferric ion to the aromatic polyhydroxy compound is 1 to 3. Preferably, the aromatic polyhydroxy compound is a compound having at least two hydroxy groups in ortho-position in relation to each other on an aromatic ring. Most preferably, it is a compound which has at least two hydroxy groups in ortho-position in relation to each other on an aromatic carbocyclic ring and which is free of exocyclic unsaturation. Included within the broad class of aromatic polyhydroxy compounds which are useful in this invention are, for example, compounds of the benzene series and of the naphthalene series, which can be represented by the formula:
where X represents the carbon atoms necessary to complete the benzene or naphthalene aromatic ring structure. In addition to the hydroxyl substituents, the aromatic ring structure can be substituted with groups such as sulfo radicals, carboxy radicals, or halogen atoms. Typical examples of aromatic polyhydroxy compounds useful in this invention include the following compounds:
pyrocatechol,
4,5-dihydroxy-m-benzene disulfonic acid,
4,5-dihydroxy-m-benzene disulfonic acid disodium salt,
tetrabromopyrocatechol,
pyrogallol,
gallic acid,
methyl gallate,
propyl gallate,
2,3-dihydroxynaphthalene-6-sulfonic acid,
2,3,8-trihydroxynaphthalene-6-sulfonic acid.

In a preferred embodiment of this invention, the aromatic polyhydroxy compound is 5,6-dihydroxy-1,2,4-benzenetrisulfonic acid or a 5,6-dihydroxy-1,2,4-benzenetrisulfonate (also known as a catechol trisulfonate or pyrocatechol trisulfonate). These compounds can be represented by the formula:
wherein M is hydrogen or a monovalent cation such as sodium or potassium. The most preferred compound of this class is 5,6-dihydroxy-1,2,4-benzenetrisulfonic acid trisodium salt.

The 5,6-dihydroxy-1,2,4-benzenetrisulfonic acid trisodium salt is advantageously employed in photographic color developing compositions in comparison with other similar aromatic polyhydroxy compounds, such as 4,5-dihydroxy-m-benzene disulfonic acid disodium salt in that it is more stable to aerial oxidation and has much less tendency to exhibit adverse sensitometric effects. It can be prepared by oxidation of 4,5-dihydroxy-m-benzene disulfonic acid disodium salt in an alkaline solution containing sulfite. Oxidation can be accomplished by bubbling air through the solution or by reaction with a persulfate.

Aromatic polyhydroxy compounds have been used heretofore in photographic color developing compositions. Thus, for example, they are used in Heilmann, U.S. patent 3,746,544, issued July 17, 1973, in combination with aminopolycarboxylic acid sequestering agents and in Vincent et al, U.S. patent 4,264,716, issued April 28, 1981, in combination with aminopolyphosphonic acid sequestering agents.

The primary function of the aromatic polyhydroxy compound in the photographic color developing compositions of this invention is to sequester iron but it can also function to sequester other heavy metals which can also catalyze the auto-oxidation of the N,N-dialkylhydroxylamine. Thus, the aromatic polyhydroxy compound stabilizes the developing composition and enables the N,N-dialkylhydroxylamine to effectively perform its function as an anti-oxidant which protects the primary aromatic amino color developing agent.

As described hereinabove, the novel color developing compositions of this invention contain at least one sequestering agent which functions to sequester calcium and thereby prevent the formation of unwanted precipitates. The preferred sequestering agent for this purpose is an aminopolycarboxylic acid sequestering agent.

The aminopolycarboxylic acid sequestering agents are well known and widely used in photographic processing. Typical examples of the aminopolycarboxylic acid sequestering agents include:
nitrilotriacetic acid, (NTA),
ethylenediaminetetraacetic acid, (EDTA),
1,3-diamino-2-propanol-N,N,N′,N′-tetraacetic acid, (DPTA),
diethylenetriaminepentaacetic acid (DTPA),
N,N′-bis(2-hydroxybenzyl) ethylenediamine-N,N′-diacetic acid (HBED),
hydroxyethylethylenediaminetriacetic acid,
cyclohexanediaminotetraacetic acid,
aminomalonic acid.

The photographic color developing compositions of this invention are employed in the form of aqueous alkaline working solutions having a pH of above 7 and most typically in the range of from about 9 to about 13. To provide the necessary pH, they contain one or more of the well known and widely used pH buffering agents, such as the alkali metal carbonates or phosphates. Potassium carbonate is especially useful as a pH buffering agent.

As indicated above, the four essential components of the novel photographic color developing compositions of this invention are the primary aromatic amino color developing agent, the N,N-dialkylhydroxylamine, the sequestering agent which functions to sequester iron and the sequestering agent which functions to sequester calcium. The N,N-dialkylhydroxylamine is preferably employed in an amount of from about 1.5 to about 6.0 moles per mole of the developing agent, the sequestering agent which functions to sequester iron is preferably employed in an amount of from about 0.04 to about 0.25 moles per mole of the developing agent, and the sequestering agent which functions to sequester calcium is preferably employed in an amount of from about 0.3 to about 1.7 moles per mole of the developing agent.

A small amount of sulfite can optionally be incorporated in the developing compositions of this invention to provide additional protection against oxidation. In view of the fact that sulfite competes with coupler for oxidized developing agent, the amount of sulfite is in the range of from zero to 0.2 moles per mole of primary aromatic amino color developing agent. The use of a small amount of sulfite is especially desirable when the color developing composition is packaged in the form of a concentrated solution, since such concentrates are especially susceptible to oxidation.

A further ingredient which can optionally be included in the color developing composition is an alkanolamine. The alkanolamines are primarily useful in providing additional protection against oxidation. As described in Case et al, U.S. patent 4,170,478, issued October 9, 1979, preferred alkanolamines for use in photographic color developing compositions are compounds of the formula:
wherein R₁ is an hydroxyalkyl group of 2 to 6 carbon atoms and each of R₂ and R₃ is a hydrogen atom, an alkyl group of 1 to 6 carbon atoms, an hydroxyalkyl group of 2 to 6 carbon atoms, a benzyl radical, or a
wherein n is an integer of from 1 to 6 and each of X and Y is a hydrogen atom, an alkyl group of 1 to 6 carbon atoms or an hydroxylalkyl group of 2 to 6 carbon atoms. Alkanolamines which are especially preferred are compounds of the formula:
wherein R₄ is an hydroxyalkyl group of 2 to 4 carbon atoms and each of R₅ and R₆ is an alkyl group of 1 to 4 carbon atoms or an hydroxyalkyl group of 2 to 4 carbon atoms. Typical examples of alkanolamines which can be used in the color developing compositions of this invention include:
ethanolamine
diethanolamine
triethanolamine
di-iaopropanolamine
2-methylaminoethanol
2-ethylaminoethanol
2-dimethylaminoethanol
2-diethylaminoethanol
1-diethylamino-2-propanol
3-diethylamino-1-propanol
3-dimethylamino-1-propanol
isopropylaminoethanol
3-amino-1-propanol
2-amino-2-methyl-1,3-propanediol
ethylenediamine tetraisopropanol
benzyldiethanolamine
2-amino-2-(hydroxymethyl)-1,3-propanediol.

To improve the clarity of the working developing solution and reduce the tendency for tarring to take place, it is preferred to incorporate therein a small amount of a water-soluble sulfonated polystyrene. The sulfonated polystyrene can be used in the free acid form or in the salt form. The free acid form of the sulfonated polystyrene is comprised of units having the formula:
where X is an integer representing the number of repeating units in the polymer chain and is typically in the range from about 10 to about 3,000 and more preferably in the range from about 100 to about 1,000.

The salt form of the sulfonated polystyrene is comprised of units having the formula:
where X is as defined above and M is a monovalent cation, such as, for example, an alkali metal ion.

The sulfonated polystyrenes utilized in the developing compositions of this invention can be substituted with substituents such as halogen atoms, hydroxy groups, and alkyl groups. For example, they can be sulfonated derivatives of chlorostyrene, alpha methyl styrene, vinyl toluene, and the like. Neither the molecular weight nor the degree of sulfonation are critical, except that the molecular weight should not be so high nor the degree of sulfonation so low as to render the sulfonated polystyrene insoluble in aqueous alkaline photographic color developing solutions. Typically, the average degree of sulfonation, that is the number of sulfonic acid groups per repeating styrene unit, is in the range from about 0.5 to 4 and more preferably in the range from about 1 to about 2.5. A variety of salts of the sulfonated polystyrene can be employed, including, in addition to alkali metal salts, the amine salts such as salts of monoethanolamine, diethanolamine, triethanolamine, morpholine, pyridine, picoline, quinoline.

The sulfonated polystyrene can be used in the working developer solution in any effective amount. Typically, it is employed in amounts of from about 0.05 to about 30 grams per liter of developer solution, more usually in amounts of from about 0.1 to about 15 grams per liter, and preferably in amounts of from about 0.2 to about 5 grams per liter.

In addition to or in place of the aminopolycarboxylic acid sequestering agent, the photographic color developing compositions of this invention can contain an aminopolyphosphonic acid sequestering agent. The aminopolyphosphonic acid sequestering agent can be utilized in the form of a free acid or in the form of a water-soluble salt. Among the useful aminopolyphosphonic acid sequestering agents are the following:
(1) amino-N,N-dimethylenephosphonic acids of the formula:
   $\text{R³ _ N(CH₂PO₃M₂)₂}$
   wherein M is a hydrogen atom or a monovalent cation and R³ is an alkyl group, an aryl group, an aralkyl group, an alkaryl group, an alicyclic group or a heterocyclic radical, and R³ can be further substituted with substituents such as hydroxyl, halogen, an alkoxy group, a _PO₃M₂ group, a _CH₂PO₃M₂ group, or an _N(CH₂PO₃M₂)₂ group;
(2) aminodiphosphonic acids of the formula: in which R⁴ is an alkyl group, preferably of one to five carbon atoms, and
(3) N-acylaminodiphosphonic acids of the formula: where R⁵, R⁶ and R⁷ are hydrogen or an alkyl group, preferably alkyl of one to five carbon atoms.

Typical examples of the aminopolyphosphonic acid sequestering agents useful in the novel color developing compositions of this invention include:
1-aminoethane-1,1-diphosphonic acid,
1-aminopropane-1,1-diphosphonic acid,
N-acetyl-1-aminoethane-1,1-diphosphonic acid,
ethylenediamine-N,N,N′,N′-tetramethylenephosphonic acid,
nitrilo-N,N,N-trimethylenephosphonic acid,
1,2-cyclohexanediamine-N,N,N′,N′-tetramethylenephosphonic acid,
o-carboxyanilino-N,N-dimethylenephosphonic acid,
propylamino-N,N-dimethylenephosphonic acid,
4-(N-pyrrolidino)butylamine-N,N-bis(methylene phosphonic acid,
1,3-diaminopropanol-N,N,N′,N′-tetramethylenephosphonic acid,
1,3-propanediamine-N,N,N′,N′-tetramethylenephosphonic acid,
1,6-hexanediamine-N,N,N′,N′-tetramethylenephosphonic acid,
o-acetamidobenzylamino-N,N-dimethylenephosphonic acid,
o-toluidine-N,N-dimethylenephosphonic acid,
2-pyridylamino-N′,N′-dimethylenephosphonic acid,
diethylenetriamine pentamethylenephosphonic acids.

Other particularly useful sequestering agents for photographic color developing compositions are the hydroxyalkylidenediphosphonic acid sequestering agents of the formula:
where R is alkyl of 1 to 5 carbon atoms.

The hydroxyalkylidenediphosphonic acid sequestering agents can serve as both the sequestering agent which functions to sequester iron and the sequestering agent which functions to sequester calcium, as they have the ability to effectively sequester both iron and calcium. As described in Brown, U.S. Patent 3,839,045 issued October 1, 1974, they are preferably utilized in combination with small amounts of lithium salts, such as lithium sulfate.

Additional ingredients which can optionally be included in the photographic color developing compositions of this invention include thickening agents, brightening agents, wetting agents, stain reducing agents, and so forth.

The photographic color developing compositions of this invention are preferably free, or at least substantially free, of bromides. By the term "substantially free" is meant a concentration of bromide of not more than about 0.01 moles per mole of primary aromatic amino color developing agent. As is well known, bromides are very active development restrainers. To achieve the objective of a very short development time, it is necessary to have little or no bromide in the developing solution. Where the emulsions used are all-chloride emlsions, then there will not be any bromide present in the developing solution as a result of leaching from the element. As previously explained herein, high chloride silver halide elements are elements in which the silver halide grains are at least 80 mole percent silver chloride. Thus, while high chloride silver halide elements can contain small amounts of silver bromide or silver bromoiodide, the amounts are low enough that the concentration of bromide in the developing solution that results from leaching is low, and the restraining effect is not pronounced.

Chloride will, of course, be leached from high chloride silver halide elements, but chloride is not nearly as active a development restrainer as bromide. An important objective of the preferred embodiments of this invention is to have minimal development restraint from either developing composition components or from seasoning products that leach from the photographic element. Thus, while the working solution may contain chloride that has leached from the element, typically no chloride is incorporated in the replenisher solution.

It is particularly preferred that the photographic color developing compositions of this invention be free of benzyl alcohol. In the past, benzyl alcohol has typically been used in the processing of color print papers to function as a coupling accelerator. Since the developing compositions of this invention are designed to have minimal development restraint _ and since oxidation protection is provided by use of an N,N-dialkylhydroxylamine, optionally with the additional use of a small amount of sulfite, and therefore without introducing significant competition with coupler for oxidized developing agent _ they do not require the use of benzyl alcohol. Elimination of benzyl alcohol has several benefits. For example, it provides improved mixability of the developing composition components and it provides the environmental improvement of reduced biological oxygen demand. A further advantage is that for those processes in which a bleach-fix is utilized, the elimination of benzyl alcohol from the developer enables the pH of the bleach-fix to be reduced without the risk of producing leuco cyan dye. The reduced pH increases the rate of bleach-fix reactions, and thereby allows a very short bleach-fix time and, accordingly, facilitates accomplishment of the goal of a very short total processing time. Yet another advantage of eliminating benzyl alcohol from the color developing composition is that this will help in avoiding or minimizing edge staining of the photographic print, as described for example in Tamagawa et al, United States Patent 4,433,030, issued February 21, 1984.

In the production of color photographic images, it is necessary to remove the silver image which is formed coincident with the dye image. This can be done by oxidizing the silver by means of a suitable oxidizing agent, commonly referred to as a bleaching agent, in the presence of halide ion followed by dissolving the silver halide so formed in a silver halide solvent, commonly referred to as a fixing agent. Alternatively, the bleaching agent and fixing agent can be combined in a bleach-fixing solution and the silver removed in one step by use of such solution.

Color print papers are most commonly processed by use of a bleach-fixing solution. The bleaching agent is typically a ferric complex of an aminopolycarboxylic acid, most usually the ferric complex of ethylenediaminetetraacetic acid (EDTA). The fixing agent is typically a thiosulfate such as sodium thiosulfate or ammonium thiosulfate.

In processing color print papers, the bleach-fixing step can be followed by a stabilizing step in which the print is processed in a stabilizing bath to reduce fading of the dye images and staining of the print that can result from exposure to high humidities and/or high temperatures. The stabilizing bath will typically contain an aldehyde, such as formaldehyde, which is known to react with the active methylene groups on residual color-forming couplers, and thus prevent them from reacting with the image dyes. In addition to the aldehyde, the stabilizing bath can contain a variety of other agents such as sequestering agents, buffering agents, and biocides. Particularly, effective stabilizing baths for use in the process of this invention are described in Mowrey, U.S. patent 3,676,136, issued July 11, 1972.

The novel color developing compositions of this invention are especially useful in the processing of color print papers utilizing high chloride silver halide emulsion layers and particularly in the processing of such papers in a rapid access process comprising the steps of color developing, bleach-fixing without a wash step between the steps of color developing and bleach-fixing, and stabilizing without a wash step between the steps of bleach-fixing and stabilizing. The bleach-fixing composition is comprised of a thiosulfate fixing agent and a ferric complex of an aminopolycarboxylic acid, which acts as a bleaching agent, while the stabilizing composition contains an aldehyde as the stabilizing agent. Such a process involves only the three steps of color developing, bleach-fixing and stabilizing _ followed by a short drying step _ so it is especially well adapted to the very short total processing time that is needed in so-called "mini-lab" processing facilities. The wash steps are omitted in the interest of achieving the shortest possible total processing time and reducing the total amount of effluent.

The present invention futhermore provides a method of rapid access processing of a high chloride silver halide photographic color print paper, which comprises the steps of:
(1) developing for a period of 30 to 60 seconds at a temperature of 30 to 40°C in a color developing composition having a pH in the range of from 9 to 13, wherein said colour developing composition in the compostition of Claim 1.
(2) bleach-fixing, without washing between the developing and bleach-fixing steps, for a period of 30 to 60 seconds at a temperature of 25°C to 40°C in a bleach-fix composition having a pH in the range of from 5 to 8 and more preferably in the range of from 6 to 7 and comprising a thiosulfate fixing agent and a bleaching agent which is a ferric complex of an aminopolycarboxylic acid;
and (3) stabilizing, without washing between the bleach-fixing and stabilizing steps, for a period of 60 to 120 seconds at a temperature of 25 to 40°C in a stabilizing compostition having a pH in the range from 5 to 8 and comprising an aldehyde hat functions as a stabilizing agent.

Following completion of the stabilizing step, the print is dried for a brief period. Drying for about one minute at a temperature of about 60°C is usually adequate.

Since, in the preferred process of this invention, no washing steps are utilized, there is carry-over of bleach-fixing composition into the stabilizing bath. The Thiosulfate which is thereby carried into the stabilizing bath can undergo sulfurization. However, the tendency for sulfurization to occur can be eliminated, or at least reduced, by use of a stabilizing bath containing an aldehyde bisulfile adduct, such as those described in Mowrey, U.S. patent 3,676,136. In addition to the aldehyde bisulfile adduct, the stabilizing bath advantageously comprises an aminopolycarboxylic acid sequestering agent, of the type hereinbefore described, and an aminopolyphosphonic acid sequestering agent or hydroxyalkylidenediphosphonic acid sequestering agent of the types hereinbefore described. The aminopolycarboxylic acid sequesters calcium, and thereby prevents the formation of unwanted precipitates, and also protects the sulfile against oxidation. The aminopolyphosphonic acid or hydroxyalkylidenediphosphonic acid sequesters heavy metals, such as copper and iron, and thereby prevents such metals from catalyzing the oxidation of sulfile. It also provides protection against yellowing of photographic prints caused by retained iron. Another useful ingredient in a stabilizing bath of this type is a biocide. Examples of particularly useful biocides are thiazoles such as 2-methyl-4-isothiazolin-3-one and 5-chloro-2-methyl-4-isothiazolin-3-one.

The individual ingredients employed in the photographic color developing compositions of this invention have been employed heretofore in one or other of the photographic color developing compositions described in the United States patents listed hereinabove. However, the particular combination of ingredients utilized in the color developing compositions of this invention is a novel combination, and is unexpectedly advantageous in providing a developing composition which is especially adapted for use with high chloride silver halide elements, and is particularly well adapted for use in the rapid access process described herein in which total wet processing time is as little as three minutes.

It should be particularly noted that 5,6-dihydroxy-1,2,4-benzenetrisulfonic acid has not been employed heretofore in photographic color developing compositions, and that its use (in either acid or salt form) represents an important feature of the most preferred embodiment of the present invention. As compared with similar compounds which have previously been used in color developing compositions _ such as the 4,5-dihydroxy-m-benzenedisulfonic acid described in United States patent 3,746,544 _ it provides several important advantages. Thus, for example, it has improved stability in alkaline solutions and is more stable to aerial oxidation. Moreover, it has much less of a tendency to exert adverse sensitometric effects.

It should also be noted that the N,N-dialkylhydroxylamine is utilized in the developing composition of this invention as an anti-oxidant. This is in contrast with its typical use in the prior art, for example, in United States patent 3,489,566, in which it is used primarily as a balancing developing agent, that is as an agent which reacts with exposed silver halide so as to function as an auxiliary developing agent.

In U.S. patents 4,170,478 and 4,264,716, the hydroxylamines which are used in the color developing compositions described are hydroxylamines of the formula:
where R is hydrogen or alkyl, and water-soluble acid salts thereof. Thus, the hydroxylamines in these patents are unsubstituted hydroxylamines or monoalkyl-substituted hydroxylamines. In the present invention, dialkyl-substituted hydroxylamines are utilized rather than unsubstituted hydroxylamines or mono-alkyl-substituted hydroxylamines. The dialkyl-substituted hydroxylamines have been unexpectedly found to provide satisfactory protection against oxidation, while having the advantage that they do not reduce oxidized developer before it can react to form dye, and the further advantage that they are much slower developing agents than unsubstituted hydroxylamines or mono-alkyl-substituted hydroxylamines. Thus, by using the dialkyl-substituted hydroxylamine and no sulfite, or a very low level of sulfite, competition with couplers in the dye-forming reactions is effectively avoided.

The invention is further illustrated by the following example of its practice:

A photographic color print paper of the high chloride type, as described in Atwell, U.S. patent 4,269,927 issued May 26, 1981, was processed in a three-step process consisting of a 45 second development step, a 45 second bleach-fix step and a 90 second stabilization step. Each of the three steps was carried out at a temperature of 35°C and the print was dried for one minute at 60°C. No washing steps were used in the process. The developing composition exhibited excellent stability and the process provided excellent results, even though the total wet time was only three minutes, and thus achieved the objective of high quality rapid-access processing, which is especially useful in a "mini-lab" facility. The color developing, bleach-fixing and stabilizing compositions used in the process were as follows:

### Bleach-Fixing Composition

The bleach-fixing composition had a pH of 6.2 and was comprised of ammonium thiosulfale, sodium bisulfile, and an ammonium salt of the ferric complex of ethylenediaminetetraacetic acid.

### Stabilizing Composition

The stabilizing composition had a pH of 7.2 and was comprised of formaldehyde, sodium metabisulfite, potassium hydroxide, diethylene glycol, 5-chloro-2-methyl-4-isothiazolin-3-one, the disodium salt of ethylenediaminetetraacetic acid, and 1-hydroxyethylidene-1,1-diphosphonic acid. (In this formulalion, the diethylene glycol serves as a solvent for the 5-chloro-2-methyl-4-isothiazolin-3-one).

An important feature of this invention is that there is minimal development restraint and this permits rapid access processing. Moreover, the rapid access processing does not require high development temperatures and can be achieved with development temperatures of as low as about 15°C.

## Claims

1. A photographic color developing composition which is especially useful in the development of high chloride silver halide photographic elements, said composition being substantially free of bromides and comprising:
(1) a primary aromatic amino color developing agent,
(2) an N,N-dialkylhydroxylamine,
(3) at least one sequestering agent which functions to sequester iron,
(4) at least one sequestering agent which functions to sequester calcium, and
(5) from zero to 0.2 moles of sulfite per mole of said primary aromatic color developing agent.

2. A photographic color developing composition as claimed in claim 1 wherein said sequestering agent which functions to sequester iron is an aromatic polyhydroxy compound that forms a complex with ferric ion in alkaline solution in which the molar ratio of the ferric ion to the aromatic polyhydroxy compound is 1 to 3, and said sequestering agent which functions to sequester calcium is an aminopolycarboxylic acid sequestering agent.

3. A photographic color developing composition as claimed in claim 1 wherein an hydroxylalkylidenediphosphonic acid sequestering agent is employed as both the sequestering agent which functions to sequester iron and the sequestering agent which functions to sequester calcium.

4. A photographic color developing composition as claimed in claim 2, said composition being substantially free of bromides and benzyl alcohol and comprising:
(1) a primary aromatic amino color developing agent,
(2) an N,N-dialkylhydroxylamine,
(3) an aromatic polyhydroxy compound that forms a complex with ferric ion in alkaline solution in which the molar ratio of the ferric ion to the aromatic polyhydroxy compound is 1 to 3,
(4) at least one aminopolycarboxylic acid sequestering agent,
(5) from zero to 0.2 moles of sulfite per mole of said primary aromatic color developing agent, and
(6) at least one pH buffering agent.

5. A photographic color developing composition as claimed in claim 1 additionally comprising an alkanolamine.

6. A photographic color developing composition as claimed in claim 5, wherein said alkanolamine is triethanolamine.

7. A photographic color developing composition as claimed in claim 1 additionally comprising a water-soluble sulfonated polystyrene.

8. A photographic color developing composition as claimed in claim 4, additionally comprising triethanolamine and a water-soluble sulfonated polystyrene.

9. A photographic color developing composition as claimed in claim 1 wherein the primary aromatic amino color developing agent is 4-(N-ethyl-N-2-methanesulfonylaminoethyl)-2-methyl-phenylenediamine sesquisulfate monohydrate.

10. A photographic color developing composition as claimed in claim 1 wherein said N,N-dialkylhydroxylamine has the formula wherein R³ and R⁴ represent the same or different alkyl groups of 1 to 4 carbon atoms.

11. A photographic color developing composition as claimed in claim 4 wherein said aromatic polyhydroxy compound has the formula: where X represents the carbon atoms necessary to complete a benzene or naphthalene aromatic ring structure.

12. A photographic color developing composition as claimed in claim 4 wherein said N,N-dialkylhydroxylamine is N,N-diethylhydroxylamine.

13. A photographic color developing composition as claimed in claim 11 wherein said aromatic polyhydroxy compound is 5,6-dihydroxy-1,2,4-benzenetrisulfonic acid trisodium salt.

14. A photographic color developing composition as claimed in claim 4 wherein said aminopolycarboxylic acid sequestering agent is ethylenediaminetetraacetic acid.

15. A photographic color developing composition as claimed in claim 4, and comprising:
(1) 4-(N-ethyl-N-2-methanesulfonylaminoethyl)-2-methylphenylenediamine sesquisulfate monohydrate,
(2) N,N-diethylhydroxylamine,
(3) 5,6-dihydroxy-1,2,4-benzenetrisulfonic acid trisodium salt,
(4) the disodium salt of ethylenediaminetetraacetic acid,
(5) the lithium salt of sulfonated polystyrene,
(6) triethanolamine,
(7) potassium sulfite, and
(8) potassium carbonate.

16. A method of rapid access processing of a high chloride silver halide photographic color element, said method comprising the steps of:
(1) developing said element for a period of 30 to 60 seconds at a temperature of 30°C to 40°C in a color developing composition having a pH in the range of from 9 to 13,
(2) bleach-fixing said element, without washing between the developing and bleach-fixing steps, for a period of 30 to 60 seconds at a temperature of 25°C to 40°C in a bleach-fix composition having a pH in the range of from 5 to 8 and comprising a thiosulfate fixing agent and a ferric complex of an aminopolycarboxylic acid that functions as a bleaching agent; and
(3) stabilizing said element, without washing between the bleach-fixing and stabilizing steps, for a period of 60 to 120 seconds at a temperature of from 25°C to 40°C in a stabilizing composition having a pH in the range of from 5 to 8 and comprising an aldehyde that functions as a stabilizing agent, wherein said color developing composition is the composition of claim 1.

17. A method as claimed in claim 16, wherein said color developing composition is the composition of any of claims 2, 3, 5, 10.

18. A method as claimed in claim 16, wherein said color developing composition is the composition of any of claims 4, 8, 12, 13.

19. A method as claimed in claim 18, wherein said bleach-fixing composition has a pH in the range of from 6 to 7.

20. A method as claimed is claim 18, wherein said stabilizing composition comprises an aldehyde bisulfite adduct.

21. A method as claimed in claim 18, wherein said stabilizing composition comprises a thiazole compound which functions as a biocide.

22. A method as claimed in claim 18, wherein said stabilizing composition comprises an aminopolycarboxylic acid sequestering agent, and a member selected from the group consisting of aminopolyphosphonic acid sequestering agents and hydroxyalkylidene diphosphonic acid sequestering agents.

23. A method as claimed in claim 1, wherein said high chloride silver halide photographic element is a color paper, said method comprising the steps of:
(1) developing said color paper for a period of 45 seconds at a temperature of 35°C in a color developing composition having a pH of 10,
(2) bleach-fixing said color paper, without washing between the developing and bleach-fixing steps, for a period of 45 seconds at a temperature of 35°C in a bleach-fix composition having a pH of 6 and comprising ammonium thiosulfate and the ammonium salt of a ferric complex of ethylenediaminetetraacetic acid; and
(3) stabilizing said color paper, without washing between the bleach-fixing and stabilizing steps, for a period of 90 seconds at a temperature of 35°C in a stabilizing composition having a pH of 6 and comprising formaldehyde, sodium metabisulfite, potassium hydroxide, diethylene glycol, 5-chloro-2-methyl-4-isothiazolin-3-one, the disodium salt of ethylenediaminetetraacetic acid, and 1-hydroxyethylidene-1,1-diphosphonic acid, wherein said color developing composition is the composition of claim 15.

## Patentansprüche

1. Photographische Farbentwicklerzusammensetzung, die sich besonders für die Entwicklung von photographischen Silberhalogenidelementen mit hohem Chloridgehalt eignet, und die von Bromiden praktisch frei ist, und enthält:
(1) eine aus einem primären aromatischen Amin betehende Farbentwicklerverbindung,
(2) ein N,N-Dialkylhydroxylamin,
(3) mindestens einen Komplexbildner, der Eisen komplex bindet,
(4) mindestens einen Komplexbildner, der Calcium komplex bindet, und
(5) 0 bis 0,2 Mole Sulfit pro Mol der aus einem primären aromatischen Amin bestehenden Entwicklerverbindung.

2. Photographische Farbentwicklerzusammensetzung nach Anspruch 1, in der der Komplexbildner, der Eisen komplex bindet, eine aromatische Polyhydroxyverbindung ist, die in alkalischer Lösung mit Ferriionen einen Komplex bildet, in dem das Molverhältnis von Ferriionen zu aromatischer Polyhydroxyverbindung bei 1 bis 3 liegt und in der der Komplexbildner, der Calcium komplex bindet, ein Aminopolycarbonsäure-Komplexbildner ist.

3. Photographische Farbentwicklerzusammensetzung nach Anspruch 1, in der ein HydroxyalkylidendiphosphonsäureKomplexbildner sowohl als Komplexbildner für die Komplexbindung von Eisen, als auch als Komplexbildner zur Komplexbindung von Calcium verwendet wird.

4. Photographische Farbentwicklerzusammensetzung nach Anspruch 2, die von Bromiden und Benzylalkohol praktisch frei ist und enthält:
(1) eine aus einem primären aromatischen Amin bestehende Farbentwicklerverbindung,
(2) ein N,N-Dialkylhydroxylamin,
(3) eine aromatische Polyhydroxyverbindung, die in alkalischer Lösung einen Komplex mit Ferriionen bildet, in dem das Molverhältnis von Ferriionen zur aromatischen Polyhdroxyverbindung bei 1 bis 3 liegt,
(4) mindestens einen Aminopolycarbonsäure-Komplexbildner,
(5) Null bis 0,2 Mole Sulfit pro Mol der aus einem primären aromatischen Amin bestehenden Farbentwicklerverbindung, und
(6) mindestens eine pH-Puffersubstanz.

5. Photographische Farbentwicklerzusammensetzung nach Anspruch 1, die zusätzlich ein Alkanolamin enthält.

6. Photographische Farbentwicklerzusammensetzung nach Anspruch 5, in der das Alkanolamin aus Triethanolamin besteht.

7. Photographische Farbentwicklerzusammensetzung nach Anspruch 1, die zusätzlich ein in Wasser lösliches sulfoniertes Polystyrol enthält.

8. Photographische Farbentwicklerzusammensetzung nach Anspruch 4, die zusätzlich Triethanolamin und ein in Wasser lösliches sulfoniertes Polystyrol enthält.

9. Phothgraphische Farbentwicklerzusammensetzung nach Anspruch 1, in der die aus einem primären aromatischen Amin bestehende Farbentwicklerverbindung 4(N-Ethyl-N-2-methansulfonylaminoethyl)-2-methyl-phenylendiaminsesquisulfat-Monohydrat ist.

10. Photographische Farbentwicklerzusammensetzung nach Anspruch 1, in der das N,N-Dialkylhydroxylamin der folgenden Formel entspricht in der R³ und R⁴ gleiche oder verschiedene Alkylgruppen mit 1 bis 4 Kohlenstoffatomen sind.

11. Photographische Farbentwicklerzusammesnetzung nach Anspruch 4, in der die aromatische Polyhydroxyverbindung der folgenden Formel entspricht: in der X für die Kohlenstoffatome steht, die zur Vervollständigung einer aromatischen Benzol- oder Naphthalinringstruktur erforderlich sind.

12. Photographische Farbentwicklerzusammensetzung nach Anspruch 4, in der das N,N-Dialkylhydroxylamin aus N,N-Diethylhydroxylamin besteht.

13. Photographische Farbentwicklerzusammensetzung nach Anspruch 11, in der die aromatische Polyhydroxyverbindung das Trinatriumsalz der 5,6-Dihydroxy-1,2,4-benzoltrisulfonsäure ist.

14. Photoraphische Farbentwicklerzusammensetzung nach Anspruch 4, in der der Aminopolycarbonsäure-Komplexbildner Ethylendiamintetraessigsäure ist.

15. Photographische Farbentwicklerzusammensetzung nach Anspruch 4, enthaltend:
(1) 4-(N-Ethyl-N-2-methansulfonylaminoethyl)-2-methylphenylendiaminsesquisulfat-Monohydrat,
(2) N,N-Diethylhydroxylamin,
(3) 5,6-Dihydroxy-1,2,4-benzoltrisulfonsäure, Trinatriumsalz,
(4) das Dinatriumsalz der Ethylendiamintetraessigsäure,
(5) das Lithiumsalz von sulfoniertem Polystyrol,
(6) Triethanolamin,
(7) Kaliumsulfit und
(8) Kaliumcarbonat.

16. Verfahren zur Schnellentwicklung eines farbphotographischen Silberhalogenidelementes mit hohem Chloridgehalt, mit den Stufen:
(1) Entwicklung des Elementes innerhalb einer Zeitspanne von 30 bis 60 Sekunden bei einer Temperatur von 30 bis 40°C in einer Farbentwicklerzusammensetzung mit einem pH-Wert von 9 bis 13,
(2) Bleichfixieren des Elementes, ohne Waschen zwischen den Entwicklungs- und Bleichfixierstufen innerhalb eines Zeitraumes von 30 bis 60 Sekunden bei einer Temperatur von 25 bis 40°C in einer Bleichfixier-zusammensetzung mit einem pH-Wert von 5 bis 8, enthaltend ein Thiosulfat-Fixiermittel und einen Ferri-Komplex einer Aminopolycarbonsäure, der als Bleichmittel wirkt, und
(3) Stabilisierung des Elementes, ohne Waschen zwischen den Bleichfixier- und Stabilisierungsstufen innerhalb von 60 bis 120 Sekunden bei einer Temperatur von 25 bis 40°C in einer Stabilisierungszusammensetzung mit einem pH-Wert von 5 bis 8, die einen Aldehyd enthält, der als Stabilisierungsmittel wirkt, bei dem man eine Farbentwicklerzusammensetzung nach Anspruch 1 verwendet.

17. Verfahren nach Anspruch 16, in dem man als Farbentwicklerzusammensetzung eine Zusammensetzung nach einem der Ansprüche 2,3,5 und 10 verwendet.

18. Verfahren nach Anspruch 16, in dem man als Farbentwicklerzusammensetzung eine Zusammensetzung nach einem der Ansprüche 4,8,12 und 13 verwendet.

19. Verfahren nach Anspruch 18, in dem die Bleichfixierzusammensetzung einen pH-Wert im Bereich von 6 bis 7 hat.

20. Verfahren nach Anspruch 18, in dem die Stabilisierungszusammensetzung ein Aldehyd-Bisulfitaddukt aufweist.

21. Verfahren nach Anspruch 18, in dem die Stabilisierungszusammensetzung eine Thiazolverbindung enthält, die als Biocid wirkt.

22. Verfahren nach Anspruch 18, in dem die Stabilisierungszusammensetzung einen Aminopolycarbonsäure-Komplexbildner enthält, sowie eine Verbindung, ausgewählt aus der Gruppe von Verbindungen bestehend aus Aminopolyphosphonsäure-Komplexbildnern und Hydroxyalkylidendiphosphonsäure-Komplexildnern.

23. Verfahren nach Anspruch 1 mit den Stufen:
(1) Entwicklung des Farbpapieres 45 Sekunden lang bei einer Temperatur von 35°C in einer Farbentwicklerzusammensetzung mit einem pH-Wert von 10,
(2) Bleichfixieren des Farbpapieres, ohne Waschen zwischen den Entwicklungs- und Bleichfixierstufen, 45 Sekunden lang bei einer Temperatur von 35°C in einer Bleichfixierzusammensetzung mit einem pH-Wert von 6, enthaltend Ammoniumthiosulfat und das Amoniumsalz eines Ferrikomplexes der Ethylendiamintetraessigsäure, und
(3) Stabilisierung des Farbpapieres ohne Waschen zwischen den Bleichfixier- und Stabilisierungsstufen, 90 Sekunden lang bei einer Temperatur von 35°C in einer Stabilisierungszusammensetzung mit einem pH-Wert von 7, enthaltend: Formaldehyd, Natriummetabisulfit, Kaliumhydroxid, Diethylenglykol, 5-Chloro-2-methyl-4-isothiazolin-3-on, das Dinatriumsalz der Ethylendiamintetraessigsäure sowie 1-Hydroxyethyliden-1,1-diphosphonsäure, wobei die Farbentwicklerzusammensetzung eine Zusammensetzung nach Anspruch 15 ist.

## Revendications

1. Composition photographique de révélateur chromogène, particulièrement utile pour le développement de produits photographiques aux halogénures d'argent à teneur élevée en chlorure, composition pratiquement sans bromures et comprenant:
(1) un développateur chromogène amine primaire aromatique,
(2) une N,N-dialkylhydroxylamine,
(3) au moins un sequestrant pour sequestrer le fer,
(4) au moins un sequestrant pour sequestrer le calcium, et
(5) de zéro à 0,2 mole de sulfite par mole de développateur chromogène amine primaire aromatique.

2. Composition photographique de révélateur chromogène selon la revendication 1, dans laquelle le sequestrant du fer est un composé aromatique polyhydroxy qui forme un complexe avec les ions ferriques en solution alcaline, complexe dans lequel le rapport molaire des ions ferriques au composé aromatique polyhydroxy est 1: 3 et le sequestrant du calcium est un acide aminopolycarboxylique.

3. Composition photographique de révélateur chromogène selon la revendication 1, dans laquelle on utilise l'acide hydroxyalkylidènediphosphonique pur sequestrer à la fois le fer et le calcium.

4. Composition photographique de révélateur chromogène selon la revendication 2, pratiquement sans bromures et sans alcool benzylique et comprenant:
(1) un développateur chromogène amine primaire aromatique,
(2) une N,N-dialkylhydroxylamine,
(3) un composé aromatique polyhydroxy qui forme un complexe avec les ions ferriques en solution alcaline, complexe dans lequel le rapport molaire des ions ferriques au composé aromatique polyhydroxy est 1: 3,
(4) au moins un sequestrant acide aminopolycarboxylique,
(5) de zéro à 0,2 moles de sulfite par mole de développateur chromogène amine primaire aromatique, et
(6) au moins un tampon de pH

5. Composition photographique de révélateur chromogène selon la revendication 1, comprenant de plus une alcanolamine.

6. Composition photographique de révélateur chromogène selon la revendication 5, dans laquelle l'alcanolamine est une triéthanolamine.

7. Composition photographique de révélateur chromogène selon la revendication 1, comprenant de plus un polystyrène sulfonate soluble dans l'eau.

8. Composition photographique de révélateur chromogène selon la revendication 4, comprenant de plus une triéthanolamine et un polystyrène sulfonate soluble dans l'eau.

9. Composition photographique de révélateur chromogène selon la revendication 1, dans laquelle le développateur chromogène amine primaire aromatique est le sesquisulfate monohydraté de la 4-(N-éthyl-N-2-méthane sulfonylaminoéthyl)-2-méthylphénylènediamine.

10. Composition photographique de révélateur chromogène selon la revendication 1, dans laquelle la N,N-dialkyl hydroxylamine a la formule où R³ et R⁴ sont des groupes alkyles identiques ou différents ayant de 1 à 4 atomes de carbone.

11. Composition photographique de révélateur chromogène selon la revendication 4, dans laquelle le composé aromatique polyhydroxy a la formule: où X représente le nombre d'atomes de carbone nécessaire pour compléter un noyau aromatique benzène ou naphtalène.

12. Composition photographique de révélateur chromogène selon la revendication 4, dans laquelle la N,N-dialkylhydroxylamine est la N,N-diéthylhydroxylamine.

13. Composition photographique de révélateur chromogène selon la revendication 11, dans laquelle le composé aromatique polyhydroxy est le sel trisodique de l'acide 5,6-dihydroxy-1,2,4-benzènetrisulfonique.

14. Composition photographique de révélateur chromogène selon la revendication 4, dans laquelle le sequestrant acide aminopolycarboxylique est l'acide éthylènediaminetétraacétique.

15. Composition photographique de révélateur chromogène selon la revendication 4, et comprenant:
(1) du sesquisulfate monohydraté de 4-(N-éthyl-N-2-méthanesulfonylaminoéthyl)-2-méthylphénylènediamine
(2) de la N,N-diéthylhydroxylamine,
(3) le sel trisodique de l'acide 5,6-dihydroxy-1,2,4-benzenetrisulfonique,
(4) le sel disodique de l'acide éthylènediaminetétraacétique,
(5) le sel de lithium d'un polystyrène sulfonate,
(6) de la triéthanolamine,
(7) du sulfite de potassium, et
(8) du carbonate de potassium.

16. Procédé pour le développement rapide de produits photographiques en couleurs aux halogénures d'argent à teneur élevée en chlorure, procédé comprenant les étapes suivantes:
(1) on développe le produit pendant 30 à 60 secondes à une température entre 30°C et 40°C dans une composition de révélateur chromogène ayant un pH compris entre 9 et 13,
(2) on effectue le blanchiment-fixage du produit, sans étape de lavage entre les étapes de développement et de blanchiment-fixage pendant 30 à 60 secondes à une température comprise entre 25 et 40°C dans une composition de blanchiment-fixage ayant un pH compris entre 5 et 8 et comprenant un fixateur thiosulfate et un complexe ferrique d'un acide aminopolycarboxylique comme agent de blanchiment; et
(3) on stabilise le produit, sans lavage entre les étapes de blanchiment-fixage et de stabilisation pendant 60 à 120 secondes, à une température comprise entre 25°C et 40°C dans une composition stabilisante ayant un pH compris entre 5 et 8 et comprenant un aldéhyde comme agent stabilisant, procédé dans lequel la composition de révélateur chromogène est la composition de la revendication 1

17. Procédé selon la revendication 16, dans lequel la composition de révélateur chromogène est la composition de l'une quelconque des revendications 2, 3, 5, 10.

18. Procédé selon la revendication 16, dans lequel la composition de révélateur chromogène est la composition de l'une quelconque des revendications 4, 8, 12, 13.

19. Procédé selon la revendication 18, dans lequel la composition de blanchiment-fixage a un pH compris entre 6 et 7.

20. Procédé selon la revendication 18, dans lequel la composition stabilisante comprend un additif qui est une combinaison bisulfitique d'un aldéhyde.

21. Procédé selon la revendication 18, dans lequel la composition stabilisante comprend un composé thiazole comme biocide.

22. Procédé selon la revendication 18, dans lequel la composition stabilisante comprend un sequestrant acide aminopolycarboxylique et un sequestrant choisi dans le groupe des sequestrants acides aminopolyphosphoniques et des sequestrants acides hydroxyalkylidène disphosphoniques.

23. Procédé selon la revendication 1, dans lequel le produit photographique aux halogénures d'argent à teneur élevée en chlorure est un papier couleur, procédé comprenant les étapes suivantes:
(1) on développe le papier couleur pendant 45 secondes à une température de 35°C dans une composition de révélateur chromogène ayant un pH de 10,
(2) on effectue le blanchiment-fixage du papier couleur, sans lavage entre les étapes de développement et de fixage pendant 45 secondes à une température de 35°C dans une composition de blanchiment-fixage ayant un pH de 6 et comprenant du thiosulfate d'ammonium et le sel d'ammonium d'un complexe ferrique d'acide éthylènediaminetétraacétique; et
(3) on stabilise le papier couleur, sans lavage entre l'étape de blanchiment-fixage et l'étape de stabilisation pendant 90 secondes à une température de 35°C dans une composition stabilisante ayant un pH de 7 et comprenant du formaldéhyde, du métabisulfite de sodium, de l'hydroxyde de potassium, du diéthylène glycol, de la 5-chloro-2-méthyl-4-isothiazolin-3-one, le sel disodique de l'acide éthylènediaminetétraacétique, et de l'acide 1-hydroxyéthylidène-1,1-diphosphonique, dans lequel la composition de révélateur chromogène est la composition de la revendication 15.
